

M. WEINRICH,  
METHOD OF MANUFACTURING CARBONACEOUS FILTERING MEDIUMS,  
APPLICATION FILED JUNE 21, 1918.  
1,308,826. Patented July 8, 1919.



*Inventor.*  
*Moriz Weinrich.*  
*By J. Walter Fowler.*  
*Attorney.*

# UNITED STATES PATENT OFFICE.

MORIZ WEINRICH, OF YONKERS, NEW YORK.

## METHOD OF MANUFACTURING CARBONACEOUS FILTERING MEDIUMS.

1,308,826.

Specification of Letters Patent. Patented July 8, 1919.

Application filed June 21, 1918. Serial No. 241,192.

To all whom it may concern:

Be it known that I, MORIZ WEINRICH, a citizen of the United States, residing at Yonkers, in the county of Westchester and 5 State of New York, have invented certain new and useful Improvements in Methods of Manufacturing Carbonaceous Filtering Mediums, of which the following is a specification.

10 My invention relates to a certain new and useful method of manufacturing carbonaceous filtering media and the invention consists of the method more particularly pointed out in the appended claims.

15 The object of the present invention is the manufacture of carbonaceous filtering materials from molasses, beet or cane molasses, or other impure or pure vegetable solutions containing sucrose or glucose, or both, and 20 finely powdered lime, either caustic or hydrated, to which in some instances, finely powdered materials, insoluble in water, like phosphate of lime, fullers' earth, kaolin, fire clay or other clays, kieselguhr, etc., or 25 mixtures thereof, shall be added. An intimate and uniform mixing of the molasses or other vegetable solutions with the finely powdered lime, or lime and some of the other named materials, is of prime impor-

30 tance and in order that my process may be better understood, I have illustrated in the drawing a type of apparatus which may be used and wherein the figure illustrates a sectional view partially in elevation of a mixer 35 in the form of a closed vessel having appropriate mixing agencies; but it will be understood that the invention is not limited to this or to any other type of apparatus and that the apparatus is illustrated merely to 40 disclose one embodiment of mechanism which may be used for effecting the intimate and uniform mixing of the solutions and ingredients before mentioned. To attain this result I may proceed substantially as fol-

45 lows:  
(a) When using caustic powdered lime the molasses, or other vegetable solutions, shall be unheated and have a density of about 75° Brix and the amount of lime 50 powder used shall be about 30% of the weight of the solution to which shall be added about 20% of finely powdered dry slaked lime.

In the aforesaid drawing, A, is a closed 55 vessel of appropriate size and construction, preferably cylindrical, having within it a

suitable stirring mechanism which may include the arms, b, fixed to a revolubly mounted shaft b', and operating in conjunction with other and stationary arms, a, fixed to the inside of the vessel. Connecting with one end of the vessel are two inlets, through one of which, d, the solution is introduced in measured quantities and through the other, d', the lime powder or a mixture of lime powder and some of the other named materials, is admitted, also in measured charges or quantities. The vertical shaft has means, as a pulley, through which power is applied to rotate the stirrer arms, b, and 60 by maintaining the cylinder or vessel A substantially full an intimate admixture of the solution and the powdered material is effected. In the opposite or lower end of the cylinder or vessel, A, is a gate-controlled 65 outlet, e, through which the mixed mass is allowed to run in receptacles, B, whose four sides have a draft toward the top, holding about two cubic feet each. They shall be filled to about 3 inches below their top and 70 then removed to a warmed room. Before these receptacles are filled their inside shall receive a thin coat of some lubricant, so that the mass will discharge easily when hardened.

85 After a while the caustic lime will combine with the water of the solution and at the same time with any sucrose, which may be in the solution, forming with it a sucrate of lime. By combining with the water of 90 the solution heat is developed and the whole mass will rise several inches and become hard but quite porous. The lime will decompose any glucose present but in doing so it will form likewise a very porous mass 95 with it. The reason for using in this case a mixture of caustic and dry slaked lime is that if the whole amount of lime would be in the caustic state its action on the water contents of the solution would be too violent 100 which might cause the burning of the whole mass.

When mixing with the solution a mixture of lime powder and powdered insoluble material, the solution shall be thinned to about 105 65° Brix and the proportion of the materials shall be about as follows:

100 weighed parts of a 65° Brix solution.

25 weighed parts of powdered caustic lime.

60 weighed parts of any of the other insoluble materials.

The lime used shall be freshly burned and

2  
ground into an impalpable powder. It is preferably burned in a kiln connected with the manufacturing plant since the carbonic acid gas, generated in the kiln, shall be likewise used with this process, as explained further down.

Another method of obtaining the desired results, may be stated as follows:

(b) When using dry slaked, powdered lime alone the solution shall be brought to, or near to boiling and when of a density of about 75° Brix about 60% of dry slaked lime of the weight of the solution shall be mixed into it in the same way as specified above. The lime will, at this temperature, likewise combine with any sucrose present in the solution to a sucrate of lime and will likewise decompose any glucose present. The hydrated lime will, however, not cause a rising and subsequent porosity of the mass but will harden into a dry, glassy mass.

When using additional powdered materials, mentioned above, the proportion of the various materials shall be about as follows: 100 weighed parts of a 65° Brix solution, heated to about boiling.

33 weighed parts of dry slaked lime powder.

60 weighed parts of any of the other 30 soluble materials.

Instead of dry hydrated lime a paste or a thick milk of lime may be used. In this case the solution has to be brought previously, when using lime alone, to at least 90° Brix and when using besides some of the other materials it shall be kept at about 85° Brix in order to secure the desired hard, glassy mass, which can be broken up easily into small pieces.

40 The mass in the receptacles will in both cases, of a mixture of caustic and dry slaked lime or hydrated lime alone be used, harden and dry within twenty-four hours, when they will be easily discharged by turning them over.

The mass is now broken up by suitable devices into small pieces. Any dust formed may be either taken back into the mixing apparatus or may be treated further together with the small pieces.

50 The material shall pass now to an appropriate drier, which may be heated by waste furnace gases, in which drier it shall be thoroughly dried.

55 When comminuted and dried in this way it undergoes now in kilns, of similar construction as those used in the manufacture of bone-black, the process of dry distillation. The escaping gases are to be utilized in the 60 well known way by condensation. They will produce methyl-alcohol, acetic acid, acetone, and a tar of peculiar odor and the proceeds from these products will cover a large portion of the working expenses.

65 When distillation is completed the prod-

uct shall be cooled in the same way as bone-black. If only lime has been mixed with the solution two kinds of carbonaceous filtering materials can be obtained. One kind is a pure, or almost pure, finely divided carbon 70 in which case the lime has to be now separated from the carbon, which has been formed by dry distillation from a part of the organic matters contained in the original solution. For this purpose the pieces shall 75 be dumped into a mixer equipped with a steam jacket and a double row of closely set mixing arms, the mixer having been filled previously with boiling water. The pieces will be broken up by the mixing arms into 80 small particles while the boiling water will dissolve a part of the lime.

The material is kept for 5 or 10 minutes in this mixer and then run into centrifugal machines lined with filter cloth and washed 85 with additional boiling water. It is then dumped into receptacles where it is boiled with dilute hydrochloric acid until all the remaining lime has been dissolved. It is then again run into centrifugals, lined with 90 filter cloth, washed with hot water and then steamed. After steaming the centrifugal is allowed to operate for 5 to 10 minutes whereby the carbon will be dried. It is then removed from the centrifugals and is ready 95 for use. Its decolorizing power in the filtration of sugar, glucose, and other solutions or oils is very great. Besides, it could be used to advantage in the manufacture of high grade printers' ink.

100 The second way is to convert the lime into carbonate of lime. To attain this the pieces, after having left the retorts and having been cooled, shall be put into a vessel provided with a perforated false bottom. It 105 is now washed with cold water, slightly acidulated with hydrochloric acid, in order to wash off any fine particles of lime, which may have settled on the surface of the material. This acidulated water shall be now 110 followed by enough pure cold water to cover the mass for several feet and carbonic acid gas from the lime kiln, or, if not connected with the plant, from some other source, shall be pumped beneath this perforated bottom. The gas will penetrate into the pieces and combine with the free lime present into carbonate of lime, which is insoluble in water, increasing thereby also the weight of the material. Or the false bottom may be placed 115 in the upper part of the vessel and the cooled material, coming from the retorts, shall be put in its dry state on this false bottom. The space beneath the false bottom is partly filled with water, kept hot or boiling by 120 steam injection. The carbonic acid-gas is pumped into this water so that the escaping gas, mingled with the vapors from the hot water, will penetrate through the perforations of the false bottom into the material 125 130

and convert its free lime contents into carbonate of lime. As soon as this has been accomplished the material may be washed in the same vessel with boiling water removing soluble impurities, then taken out and dried in some suitable drying device, when it will be ready for use.

Instead of converting the free lime into carbonate of lime, it may be converted, after

10 the material has been washed with acidulated water, into phosphate of lime. In this case the material is dumped into a vessel containing a hot solution of phosphoric acid strong enough to convert the free lime into 15 phosphate of lime. It is then taken out washed with boiling water and dried. I prefer, however, generally the use of carbonic acid because it costs nothing when a lime kiln is connected with the plant.

20 When manufacturing mixtures containing besides lime any of the above mentioned finely powdered insoluble materials, the pieces after having left the retorts shall be treated in the same way with carbonic acid 25 gas or a phosphoric acid solution. It will then make a cheap and effective substitute for bone-black. After each use the material can be revivified to good advantage by gentle oxidation according to my process and 30 apparatuses covered by my U. S. patents of December 15, 1914, Number 1,121,429; of May 23, 1916, Number 1,185,397; and of May 23, 1916, Number 1,184,398.

The lime or lime-stone used with this 35 process shall be of the same quality as that used generally in the sugar industry and may contain a few per cent. of impurities as silica, alumina and magnesia.

The revivification of pure carbon when 40 used for filtering purposes is done best and cheapest by boiling it in closed vessels, equipped with a condenser for condensing escaping vapors, in an ammonia solution. The ammonia will dissolve the impurities 45 and coloring matter taken up by the carbon and will then escape with the water vapors

with which it will be condensed and used over and over again. The material is then run with the remaining water into filter presses and washed therein with hot water 50 when it is again ready for use.

Having thus described my invention what I claim as new and desire to secure by Letters Patent is:—

1. The manufacture of carbonaceous filtering media consisting in mixing solutions containing sucrose or glucose or both with lime in such proportions and at such temperatures that a chemical combination of the lime and sucrose or glucose will take place 55 obtaining a hard mass; comminuting this mass; then calcining the mass; then cooling the burnt material and then preparing the same for filtering media, substantially as set forth.

2. The manufacture of carbonaceous filtering media consisting in mixing solutions containing sucrose or glucose or both with lime in such proportions and at such temperatures that a chemical combination of the lime and 60 sucrose or glucose will take place obtaining a hard mass; comminuting this mass; then calcining the mass; then cooling the burnt material, and finally converting its free lime contents by means of some suitable 65 acid into a calcium-salt insoluble in water.

3. The manufacture of carbonaceous filtering media consisting in mixing solutions containing sucrose or glucose or both with a mixture of lime and other powdered materials which latter are insoluble in water, the mixture being in such proportions and at such temperatures that a chemical combination of the lime and sucrose or glucose will take place obtaining a hard mass; comminuting this mass; then calcining the mass; cooling the burnt material and finally converting its free lime contents by means of some suitable acid into a calcium-salt 80 insoluble in water.

In testimony whereof I affix my signature.  
MORIZ WEINRICH.